# EUROPEAN PATENT SPECIFICATION

(11) **EP 2 337 875 B1**
(45) Date of publication and mention of the grant of the patent: **23.08.2017**
(21) Application number: 09782581.4
(22) Date of filing: 03.09.2009
(51) Int. Cl.: C23C 4/02, C23C 4/073, F01D 5/00, F01D 5/28, C25F 5/00

(54) **METHOD FOR THE RESTORATION OF A METALLIC COATING**
VERFAHREN ZUR WIEDERHERSTELLUNG EINES METALLISCHEN ÜBERZUGES
PROCÉDÉ POUR LA CONFIGURATION DES SERVICES D'UN RÉSEAU PERSONNEL

(30) Priority: 19.09.2008 EP 08164681
(43) Date of publication of application: 29.06.2011
(73) Proprietor: Ansaldo Energia Switzerland AG, 5401 Baden (CH)
(72) Inventor: BECKEL, Daniel, CH-5430 Wettingen (CH); STANKOWSKI, Alexander, CH-5301 Siggenthal-Station (CH); REITZ, Daniel, CH-5034 Suhr (CH)
(74) Representative: Bernotti, Andrea
(86) International application number: PCT/EP2009/061422
(87) International publication number: WO 2010/031696

(56) References cited:
- EP-A- 1 010 782
- EP-A- 1 094 134
- EP-A- 1 408 134
- EP-A- 1 798 302
- EP-A- 1 927 677
- US-A1- 2002 066 770
- US-A1- 2003 167 616
- US-A1- 2005 235 493
- US-A1- 2006 001 420

## Description

### TECHNICAL FIELD

The present invention relates to the field of restoration of coated components of gas turbines wherein the coatings include metallic coatings and coating systems having at least a metallic coating and wherein the coating that has to be restored includes a consumed portion. Throughout this specification the term metallic coating is used to generically describe metallic overlays, diffusion and bond coatings.

### BACKGROUND OF THE INVENTION

Components such as turbine blades, vanes or structural parts operating in the hot gas path environment of a gas turbine engine can be subjected to high temperature, thermal cycling as well as degrading environments that promote oxidation and corrosion. In order to prevent or at least minimise oxidation and hot gas corrosion it is common practice to apply a metallic coating or a combination of a metallic and a ceramic coating to the surface of the component, wherein the ceramic coating is a thermal barrier coating (TBC). The coatings can result in improved efficiency of the engine by enabling an increase in operating temperatures or alternatively a reduction in cooling air consumption.

Protective coatings can comprise a metallic coating applied to the component surface, to form a bond coating, or inner metallic coating, and an insulating ceramic outer layer, applied directly onto the bond coat, to form a TBC outer coating that can be made of zirconia stabilized with yttria. Alternatively only metallic coatings can be formed, also in combinations with other coatings.

Ni, Al and Cr, or Co, Ni, Al and Cr or Pt and Al based alloys can be used to form metallic coatings. Coatings can also take the form of MAl wherein M is at least one element selected from Fe, Ni, and Co and comprises, for example MAl, MAlY, MCrAl, MCrAlY. Another class of coatings are diffused aluminide coatings. The coatings may consist of one or more layers distinguished by their chemical or physical properties, and e.g. one layer of the metallic coating system is of MCrAI(X) type, where M is an element selected from the group containing Ni, Co, Fe and combinations thereof; X is an element selected from the group consisting of Y, Ta, Si, Hf, Ti, Zr, B, C and combinations thereof. Another possibility is that one layer of the metallic coating can be an aluminide, noble-metal-aluminide, noble metal-nickel-aluminide or the like.

The metallic coatings can be applied by vapour deposition, such as PVD, CVD, or thermal spray methods, atmospheric spray methods, sputtering, cathodic arc, and electron beam, as well as by plasma spray processes. Coating composition, microstructure and thickness are controlled by processing parameters. Diffused aluminide coatings have been applied by a variety of methods including, as used in the art, pack cementation, above the pack, vapour phase, chemical vapour deposition and slurry coating processes. The thickness and composition of the end product coating can be controlled by varying coating time, coating temperature and activity of the coating materials and process. Incorporating such elements as Pt, Rh, Pd, Cr, Si, Hf, Zr, and/or Y often enhances the performance of such coatings. With either type of metallic coating, elements of the coating interdiffuse with an article substrate during processing or operation or both yielding a diffusion zone between the metallic coating and the underlying article substrate. The diffusion zone is considered to be part of the metallic coating. As used herein, the term inner metallic coating is intended to mean at least a portion of the remaining inner metallic coating and such diffusion zone between the metallic coating and the underlying article substrate.

For gas turbine engine applications, the materials and processing methods chosen for the coating system are selected to provide resistance to spallation of the ceramic outer layer during thermal cycling of the engine as well as resistance to the oxidizing and corrosive environment in the case of a spallation event. During normal engine operation after time, the coatings, including the metallic coating and the ceramic outer layer, will degrade (preferably or particularly) in certain surface areas most subject to operating conditions and environmental stress, the degradation may also depend on the local quality of the coating at these locations. The metallic coating has been observed to be consumed by thermally grown oxides (degradation), consumption of reservoir phases and it has been observed to interdiffuse with a component substrate in such surface areas during operation to the extent that its protective ability has been reduced below an acceptable level, necessitating the removal and reapplication of a protective coating. Therefore, throughout this specification the term consumed portion of the metallic coating is used to describe that part of the metallic coating that is consumed by above-described processes including degradation, depletion (consumption of reservoir phases) and interdiffusion. The consumed portion represents the amount of the metallic coating that has been consumed.

A current practice in such repair is to remove the entire coating including the metallic coating, optionally along with its zone of diffusion with the component substrate, and the outer ceramic layer. This usually leads to a reduction of the wall thickness. After any required repair of the component structure, the entire coating, including a new metallic coating and a new outer ceramic coating, is reapplied. However, that type of coating system removal, in which the metallic coating is removed, will lead to thinning of component walls and reduce the number of possible repairs of the component, which is an undesirable cost factor. Further the complete removal increases throughput time for the repair process.

Stripping techniques disclosed in the prior art are not fully satisfactory, insofar as normally the entire coating is removed before a new coating can be applied, irrespective if the entire coating was consumed or not, or if the coating degradation was inhomogeneously distributed over the component surface. This is expensive and bears the risk of reducing the wall thickness of the underlying base material, since the base material is exposed to the abrasive treatment or aggressive stripping media prior to, subsequent or combined with mechanical treatment. Furthermore, reapplying the entire coating thickness is also more expensive and requires more time than replacing only the consumed portion of the coating.

US 4339282 and US 4944807 for example disclose specific etching baths into which the component of which the coating is to be removed can be immersed. In both cases the aim is to remove the full coating structure of the whole component in order to apply a new coating afterwards.

US 4894130 discloses a method for removal of such coatings in which the cleaned and activated component is immersed into an electrolyte bath and removal of the full coating layer takes place by applying an electric potential between the component and a cathode.

Another approach, disclosed in the prior art, involves local repair of coatings. US 6042880 for example discloses a method for complete removal of the ceramic TBC layer in local areas only in a manner such that the bond coat layer, i.e. the metallic coating layer is essentially not affected by the removal process and therefore does not have to be completely reconstituted. Another method is disclosed in EP 0713957, here the entire coating structure is completely removed from certain areas such that the actual component material is uncovered and subsequently in these areas a new coating is built up.

This is appropriate if the coating is only deteriorated in a discrete location.

However, in general the metallic coating on the entire component surface is affected to some degree, since the entire component surface is exposed to the hot gas during operation of the gas turbine. Consequently, even when an inhomogeneous distribution of coating deterioration is present, the coating is consumed to some degree on the entire surface, but not within the entire thickness.

Most of the processes known from the state-of-the-art (see for example US 2005/0235493, EP 1 798 302, EP 1 927 677, EP 1 408 134) deal with situations where after visual inspection, which only allows to determine true local damages but not the actual consumed portion of a coating. Subsequently the entire coating thickness is removed only in the locations, which have been visually determined before. Removal is done using mechanical grinding or other mechanical removal techniques and the metallic coating is subsequently restored. These processes do not just remove the consumed portion of a metallic coating but they are actual local damage repair processes.

Therefore, a technique, which is able to restore the consumed portion of the coating, over the entire coated area, would be of great benefit.

The prior art processes lack the following features:
- A simple and cheap method to determine the thickness (e.g. amount) of consumed portions of the coating, that require replacement;
- A method for removing the coating, that can be controlled to such an extent that only the consumed portion of the coating is removed and the underlying substrate is not affected. This decreases the number of potential restoration processes.
- A means of assessing the overall coating quality after restoration of the coating with undamaged inner coatings.

A combination of these three points is necessary for successful and economic application of customized coating restoration.

### SUMMARY OF THE INVENTION

The object of the present invention is therefore to provide an improved, simple and cheap method for the restoration of consumed portions of coatings of the above type, applied to metallic components, for example of gas turbines or combustion chambers. In particular the present invention relates to restoration of normally just the outer portion of coatings for components with undamaged inner portions of coatings and intact substrate (base metal).

The present invention correspondingly provides the method of claim 1 for restoration of a consumed portion of a metallic coating or a metallic coating system of a component. One of the concepts of the present invention consists in a targeted manner, in a first step, of determining in detail where the metallic coating is consumed, to what extent (up to which thickness) it is consumed and if it needs to be replaced. Correspondingly in this first step the component to be restored is analysed and the amount of consumed metallic coating which is to be replaced (the thickness thereof) is determined, preferably in spatially resolved manner, i.e. in a manner such that the consumed portions of the metallic coating are identified as a function of the location on the component.

In a second step, again in a targeted manner, based on the collected data in the first step, the consumed portion of the metallic coating is removed, only to the extent (thickness) as necessary. Normally in this step the entire thickness of the metallic coating is not removed but rather only a fraction thereof, which is exposed towards the surface side. Normally in this step at least the diffusion zone of the metallic coating layer remains intact.

Subsequently, a new metallic coating portion is applied onto the component to where the consumed portion of the metallic coating has been removed in a manner at least compensating for the coating removed in the previous step. The new metallic coating can be applied over the entire surface areas to be coated. The application of new metallic coating is preferably tailored such that the amount of coating applied is a function of the location so as to compensate for the coating removed in the second step. The final target of this third step is to reconstitute the metallic coating layer so as to be homogeneous and intact to an extent that, for example, an optional ceramic thermal barrier coating can be applied as a top coating.

It is one particular gist of the present invention to remove the metallic coating on the entire coated surface of the component. In other words wherever a metallic coating is present on the component at all (sometimes parts of the component such as the root sections are not coated), it shall be at least partially removed, typically not the whole thickness but a fraction thereof. The removed amount is not the same for the entire coated surface, but it depends as a function of location on the component, based on the result of an identification step, in which the consumed portion (the necessary removal thickness) of the metallic coating is determined using non-destructive analysis techniques as a function of location on the component. Typically this is not possible visually but needs to be carried out by specific methods as outlined below. Alternatively, or in addition to that, it is possible to determine the necessary removal thickness as a function of location using destructive techniques on representative components.

According to the invention, this removal of the metallic coating in a varying thickness as a function of location on the component takes place using electrolytic stripping. This is done by using specifically tailored counter electrodes, wherein the tailoring of the counter electrodes is carried out in accordance with the results of the identification step. In a nutshell this means that the counter electrode is structured and/or spatially arranged with respect to the component such that the electrical field between the component and the counter electrode as well as the corresponding removal process depends on the location. The aim is to remove as little as possible but as much as necessary of the metallic coating as identified in the identification step. Generally, the metallic coating is used/consumed on the entire component surface at least partially;, therefore typically wherever metallic coating is present on the component it will be at least partially removed in this process. However, preferably it will at no location be completely removed, if not absolutely necessary, such that preferentially the diffusion zone remains intact.

In contrast to the state-of-the-art, where after visual inspection of true local damages local removal of the metallic coating and subsequent restoration thereof takes place, the presently proposed method is a particularly tailored method for partially (i.e. not entire thickness) coating removal from the entire surface. The removal of the metallic coating on the location, i.e. depending on the location the metallic coating will be removed only to a limited extent, up to substantially, preferably however at no location completely.

In an optional fourth step of the proposed method the quality of the reconstituted (metallic) coating is checked. If during this step a quality defect is found, step c. can be repeated.

As mentioned above, preferentially wherever metallic coating is present on the component, it is at least partially removed in step b. leading to an at least partial reduction of the thickness of the entire metallic coating on the component as a result of step b..

It should generally be noted that prior to carrying out the above method should a ceramic coating layer be present on top of the metallic coating layer, optionally the component can be prepared by removal of this ceramic coating layer. The removal of the ceramic (thermal barrier) coating layer is normally carried out by using mechanical or chemical removal methods. One method is for example grit blasting of the component to remove the ceramic coating layer. After the removal of the ceramic coating layer normally the component is rinsed and cleaned. If necessary cleaning can be supplemented by chemical cleaning treatments for example by immersion into an acid bath and/or an alkaline bath.

As concerns the removal step b. this can be followed by a cleaning step (rinsing, brushing and the like) and prior to the initiation of the deposition step c. for the new metallic layer the exposed surface can be prepared/activated by chemical and/or mechanical methods.

According to the invention, in step a. the amount, and/or also the condition, and the associated location of total coated surface, is determined by using one or several non-destructive techniques, preferably selected from the group of: infrared thermography, X-ray fluorescence spectroscopy, ultrasonic or eddy current techniques or combinations thereof. For example an x-ray gun, which can be mounted on a robot can be used to determine by monitoring the variances in aluminium/chromium content of the coating layer whether coating is consumed or not. It should be noted that it is not necessary to carry out the identification step for each and every component to be reconstituted. It is for example in case of blades sufficient to carry out this identification step for one or a few of the blades per row, and subsequently the complete set of blades of the whole row can be subjected to the removal and reconstitution process, as the blades of a row are in a comparable condition and therefore show a similar degradation pattern.

According to the invention, in step b. the consumed portion of the metallic coating is removed by an electrolytic method comprising the steps of:
b1. immersing the component in an electrically conductive bath,
b2. electrically contacting the component and a counter electrode, in the bath,
b3. applying a potential between the component and the counter electrode, such that the component functions as an anode and the counter electrode as a cathode,
b4. controlling the potential between the anode and the cathode and measuring the current in order to monitor the coating removal or controlling the current between the anode and the cathode and measuring the voltage in order to monitor the coating removal; and
b5. stopping the coating removal of step b4. based on the monitoring of the coating removal.

Electrochemical stripping as such is known from the state-of-the-art (see for example EP 1 010 782, EP 1 094 134), however it was hitherto unknown that it would be possible to use such a process not for a complete removal of a metallic coating, but, according to the invention, very selectively only remove the consumed portion as specifically determined in an identification step carried out previously. There was no suggestion in the state-of-the-art to only remove the consumed portion of a coating and not the complete coating layer, and it was even less suggested that this would be possible by using correspondingly tailored counter electrodes.

Preferentially, the electrically conductive liquid bath is an aqueous acidic solution, preferably comprising HCl. Most preferred it is an aqueous hydrogen chloride solution, i.e. an aqueous solution of HCl, which contains 2-30 mass % hydrogen chloride.

Preferably at least when the potential is applied, the electrically conductive liquid bath has a temperature between room temperature and 80°C. It is further preferred that the electrically conductive liquid bath contains one or more of the following additional constituents: accelerators, inhibitors, pH buffers, anti-settling agents, anti-foaming agents, dispersants, wetting agents, surfactants and stabilizers.

Furthermore, the electrically conductive bath can be agitated at least when the potential is applied.

According to a further embodiment, either during step b. or subsequent to step b. the amount (i.e. the thickness), and/or the condition and the associated location of the total coated surface is determined by using one or several non-destructive techniques, preferably selected from the group of: infrared thermography, X-ray fluorescence spectroscopy, ultrasonic or eddy current techniques or combinations thereof.

According to a still further preferred embodiment of the proposed method, in step c. the new coating is applied to a thickness (identifying the consumed portion) as determined in step a. by a thermal spray technique, a gas phase deposition such as chemical or physical vapour deposition or modifications thereof, or a slurry technique or combinations/sequences of these methods.

Preferably, the thermal spray technique is high velocity oxy fuel spraying, atmospheric plasma spraying, vacuum plasma spraying or low vacuum plasma spraying.

Preferentially, in step d. the quality of the restored metallic coating is controlled by non-destructive techniques. These non-destructive techniques can for example be selected from the group of: thermography, X-ray fluorescence spectroscopy, ultrasonic or eddy current techniques or combinations thereof. Preferably, the same method and apparatus is used as is used for step a.

As mentioned above, typically the component is a gas turbine component (blade, vane, structural parts, etc). Typically such a gas turbine component consists of a Ni, Co, or Fe based superalloy or of a Ti based superalloy or of combinations thereof.

It is possible that the proposed method is applied in a situation where the coating consists of one or more layers which are distinguished by their chemical or physical properties, wherein preferably at least one layer of the metallic coating is of MCrAI(X) type, where M is an element selected from the group containing Ni, Co, Fe and combinations thereof; X is an element selected from the group consisting of Y, Ta, Si, Hf, Ti, Zr, B, C and combinations thereof and/or wherein at least one layer of the metallic coating system is an aluminide, noble-metal-aluminide, noble metal-nickel-aluminide or combinations thereof.

As mentioned above, it is preferred that the new coating is applied in a manner compensating for the removed consumed portion of the coating. This is made possible by configuring and arranging of, in step b., the geometry and/or the material of the counter electrode in such a way that metallic coating is mainly or selectively removed in the locations determined in step a. This is preferably possible by the configuring and arranging of the geometry of the counter electrode such that the distance between counter electrode and the article is larger in locations where less coating shall be removed. The size and/or the structure/surface and/or the position and/or the topology and/or the grid structure/width of the counter electrode can also be adjusted in locations where less or more coating shall be removed. It is for example possible to use a grid or web like counter electrode which allows to adapt the current density on the one hand by adaptation of the grid width and/or by the adjustment of the distance to the surface to be treated. Another advantage associated with the use of a grid or web like counter electrode is the fact that it allows a much more efficient agitation of the stripping medium to achieve a fast and homogeneous stripping reaction.

In addition to this method, it is possible to prior to step b. mask the component such that the metallic coating is selectively exposed in the regions where consumed portions have to be removed during the step b., i.e. in the locations as determined in step a.. Electroplater's tape, clip-on tooling, inert coatings etc can for example, effect such a masking.

It is not only possible to remove metallic coating by using electrolytic processes, but also to apply the new coating using galvanic deposition. Along this line, according to another embodiment of the proposed method, in step c. the new coating is applied with a thickness as determined in step a. using a galvanic deposition process. Also in this case preferably the geometry and the material (or any other property leading to locally different adapted galvanic processes) of the counter electrode is configured and arranged such that metallic coating is selectively deposited on the locations to be reconstituted. The geometry of the counter electrode can for example be configured and arranged such that the distance between the counter electrode and the article is larger on locations where less coating shall be reconstituted (galvanically deposited) and/or the size and/or the structure/surface and/or the position and/or the topology and/or the grid structure/width of the electrode is correspondingly adapted in locations where coating shall be reconstituted. It should be noted that in cases where, for the removal of the coating, an electrolytic process was already used using a specifically tailored counter electrode, that same counter electrode geometry can be used, for the deposition process, as a cathode leading to homogeneous coating thickness restoration.

Further embodiments of the present invention are outlined in the dependent claims.

### SHORT DESCRIPTION OF THE FIGURES

In the accompanying drawings preferred embodiments of the invention are shown in which:
- Figure 1: is a flow diagram of the steps of the proposed method;
- Figure 2: is a schematic diagram of a cross section of a coated component after operation in a gas turbine;
- Figure 3: is a cross sectional view of a coated component after operation in a gas turbine;
- Figure 4: is a cross section view of the coated gas turbine component shown in Figure 2 after selective removal of the consumed portion of the coating;
- Figure 5: is a cross section view of the gas turbine component displayed in Figure 4 after application of new coating; and
- Figure 6: is a cross sectional view of a micrograph of a gas turbine component with a coating on the component surface wherein the coating includes several layers and was restored as described in the present innovation in a gas turbine refurbishment.

### DETAILED DESCRIPTION OF THE PREFERRED EMBODIMENTS

Generally stated, the present invention provides a customized repair that overcomes the problems inherent to prior art and involves the following steps:
a. Identifying the portion of the coating, which is consumed as a function of location on the component. This is achieved by one or more non-destructive techniques such as, but not limited to: thermography, X-ray fluorescence spectroscopy, ultrasonic or eddy current investigations. The integrity of the component below the coating can be verified using the same methods. Alternatively, in order to assess coating quality representative members of one row of components can be additionally investigated by destructive techniques.
b. Removing by means of a process at least the consumed portions of the coating, preferably only the consumed portion. According to the invention, this is achieved by electrolytic stripping, i.e. immersing the component in an electrolytic bath and applying a potential between the component (anode) and a cathode. The electric current (or the voltage depending on the control) changes during the stripping process depending on the amount and condition of overall coating. Consequently, the stripping can be stopped at the previously determined desired end point. If necessary, specific locations of the component can be protected by masking during the stripping process. This allows locally varying degrees of coating removal, according to a previously defined pattern for coating removal.
c. Applying a new coating, such that the thickness of the remaining coating, plus the thickness of the newly applied coating add up to the thickness distribution according to the component specific coating zone drawing.
d. Optionally quality controlling to verify if the coating restoration fulfils the requirements. The quality control is achieved by non-destructive techniques, as described in section a.

Referring to the drawings, which are for the purpose of illustrating preferred embodiments of the invention and not for the purpose of limiting the scope of the invention figure 1 shows in a flow diagram schematically the above steps. In italics important aspects of each step are summarised.

Figure 2 shows a schematic diagram of a cross section of a coated component (1) having a coating (2) on the surface after service in a gas turbine,. In the situation shown in this figure any ceramic thermal barrier coating on top of the metallic coating (2) has already been removed by, for example, a mechanical method such as sand blasting or grit blasting possibly supplemented by chemical methods and subsequent cleaning. The outer part (3) of the coating is oxidised and the portion below the oxidised coating is consumed (4) and requires replacement. The lower portion of the coating (5) is still in acceptable conditions and can be operated again in the gas turbine. A diffusion zone (6) is normally formed between the base material of the component (1) and the coating (2).

Figure 3 shows a corresponding cross section micrograph of a coated component (1), having a coating (2) on the surface after service in a gas turbine. The outer part (3) of the coating is oxidised and the portion below the outer part (3) is consumed (4) and requires replacement. The lower portion of the coating (5) is still in acceptable conditions and can be operated again in the gas turbine. A diffusion zone (6) is formed between the base material of the component (1) and the coating (2).

Such a component can be subjected to the proposed method using the above steps. By means of figure 4 and figure 5 it shall be illustrated what happens to the metallic coating during these steps.

After locating consumed portions of a coating, as shown in figure 2, the consumed portions of the coating are removed by immersion of the relevant parts into an electrolyte bath and by applying a cell voltage in the range of typically several thousand mV having an anodic current density in the range of 0.5-10 A/dm². The electrolyte bath is a 10-20 mass % hydrochloric acid bath at a temperature in the range of 30-50°C. The time taken for the electrolytic removal process is adapted to the amount of consumed portion of the coating to be removed. This process can for example be controlled by keeping the anodic current density constant over time and by monitoring the voltage. If the consumed portion of the coating is removed one can detect a change in the voltage and correspondingly stop the process at the optimum moment. Alternatively it is possible to keep the cell voltage constant and monitor the anodic current density. The anodic current density can also be monitored for pronounced changes that indicate that the consumed portion of the coating has been removed sufficiently to expose the metallic coating that is not consumed. The result is a situation as shown in figure 4, which is a cross section view of the coated gas turbine component (1) displayed in figure 3, after selective removal of the consumed portion of the coating. By this means only the portions of the coating, which are in acceptable condition (5) remain. A diffusion zone (6) is formed between the base material of the component (1) and the remaining coating (5).

After this the coating layer is reconstituted wherever it had been removed, leading to a situation as shown in figure 5, which shows a schematic cross section view of the gas turbine component (1) shown in figure 4, after application of a new coating (7). The entire coating (2) thickness meets the component specific coating zone drawing. A diffusion zone (6) is located between the base material of the component (1) and the coating (2).

Figure 6 finally shows a cross sectional micrograph of a gas turbine component (1) with a coating (2) on the surface of the component, the coating (2) includes several layers as described below. The coating (2) was restored as described here in a first gas turbine refurbishment. The component was again successfully operated in the gas turbine. The micrograph shows the status after completion of the second operation interval.

The inner layer (5) of the coating system (2) directly adjacent to the diffusion zone (6) on the component (1) surface is the original unrestored coating of the coating. During the restoration according to the invention a second layer (8) of coating was applied. In the second operation interval of the component in the gas turbine, the outer portion (3) of this layer was oxidised and the portion below (4') the outer portion (3) was consumed. The inner portion (5') of the second coating layer after service exposure (8) and the original coating (5) have protected the component during a second operation period.

### Experimental section:

A used gas turbine rotating blade, the substrate of which was based on a conventional superalloy (as known for example from US 4,643,782, EP 0 208 645 or EP 0 914 483) coated with a metallic coating based on MCrAlY, was subjected to the following treatment:
- the consumed portion of the entire metallic coating of the blade was determined as a function of location on the blade, wherein the identification was performed by using infrared thermography and x-ray fluorescence spectroscopy;
- only the consumed portion (i.e. only up to the thickness that was consumed) was removed as a function of the location as identified above over the entire coated surface area.
   This step was carried out using an electrolytic method by immersing the component in an aqueous acidic solution, with a concentration of HCl of approx. 12 mass % and at a temperature of 35°C, and by electrically contacting the component and a counter electrode, both immersed in the acidic bath. The geometry of the counter electrode was configured and arranged such that the distance between the counter electrode and the component was larger in locations where less coating was to be removed in accordance with the inspection step and in locations where more coating was to be removed the width of the grid structure and the distance to the counter electrode was adjusted correspondingly.
   A potential of approx. 140 mV between the component and this specifically tailored counter electrode was applied and controlled between anode and cathode during the removal process and the current was constantly measured in order to monitor the coating removal process. The coating removal was stopped based on the monitoring of the coating removal and based on the target removal thickness according to the identification step.
   After this removal treatment over the entire component surface, the metallic layer (wherever present on the component at all) was removed partially but at no place completely. The removal thickness was just as determined in the identification step.
- Subsequently, a new metallic coating was applied using electrolytic deposition and using the same counter electrode geometry as for removal in a manner just compensating for the coating removed in the preceding steps.

### LIST OF REFERENCE NUMERALS

- 1: component, substrate
- 2: metallic coating
- 3: outer oxidised part of metallic coating
- 4: consumed part of metallic coating
- 5: intact part of metallic coating
- 6: diffusion zone of metallic coating
- 7: new part (layer) of metallic coating
- 8: second coating layer after service exposure

## Claims

1. A method for restoration of a metallic coating (2) of a component (1), wherein the coating (2) includes a consumed portion (3, 4), the method comprising the steps of:
a. identifying the consumed portion (3, 4) as a function of location on the component (1), wherein the identification is performed by using one or several non-destructive techniques;
b. removing essentially only the consumed portion (3, 4) as a function of the location as identified in step a., wherein removal is carried out using an electrolytic method comprising the steps of:
b1. immersing the component in an electrically conductive liquid bath;
b2. electrically contacting the component and a counter electrode, which are immersed in said bath;
b3. applying a potential between the component and said counter electrode, such that the component functions as an anode and the counter electrode as a cathode;
b4. controlling the potential between anode and cathode and measuring the current in order to monitor the coating removal or controlling the current between the anode and the cathode and measuring the voltage in order to monitor the coating removal; and
b5. stopping the coating removal of step b4. based on the monitoring of the coating removal;
wherein in step b. the geometry and the material of the counter electrode for electrolytic removal is configured and arranged to selectively remove metallic coating (2) as a function of the location as identified in step a.,
c. applying new metallic coating (7) in a manner at least compensating for the coating removed in step b..

2. The method according to claim 1, wherein, wherever metallic coating (2) is present on the component (1), it is at least partially removed in step b. leading to an at least partial reduction of the thickness of the entire metallic coating (2) on the component (1) as a result of step b..

3. The method according to claim 1 or 2, further including after step c. the following step d.:
d. verifying the quality of the restored metallic coating (2).

4. The method according to claim 1, 2 or 3, wherein step a. further includes determining the condition of either consumed (3, 4) or unconsumed or both consumed (3, 4) and unconsumed portions of the metallic coating (2).

5. The method according to any of the preceding claims, wherein the identifying or determination of step a. is at least partly performed by using one or several non-destructive techniques, selected from the group of: infrared thermography, X-ray fluorescence spectroscopy, ultrasonic or eddy current techniques or combinations thereof.

6. The method according to any of the preceding claims, wherein the amount of metallic coating (2) to be replaced is also determined on at least one representative component by destructive techniques, such as, but not limited to, metallographic investigations.

7. The method according to any of the preceding claims, wherein the electrically conductive liquid bath is an aqueous acidic solution, preferably comprising HCl as the main active constituent, wherein preferably the concentration of HCl is in the rage of 2-30 mass %.

8. The method according to any of the preceding claims, wherein the electrically conductive liquid bath has a temperature between room temperature and 80°C, and/or wherein the electrically conductive liquid bath contains one or more of the following additional constituents: accelerators, inhibitors, pH buffers, anti-settling agents, anti-foaming agents, dispersants, wetting agents, surfactants and stabilizers.

9. The method according to any of the preceding claims, wherein the electrically conductive liquid bath is agitated at least when the potential is applied.

10. The method according to any of the preceding claims, wherein subsequent to or concomitant to step b. the amount, and/or the condition and the associated location of the total coated surface is determined by using one or several non-destructive techniques, preferably selected from the group of: infrared thermography; X-ray fluorescence spectroscopy, ultrasonic or eddy current techniques or combinations thereof.

11. The method according to any of the preceding claims, wherein in step c. the amount of the applied new coating is a function of the identification or determination of step a. and the application of the new metallic coating is by a thermal spray technique, wherein preferably the thermal spray technique is high velocity oxy fuel spraying, atmospheric plasma spraying, vacuum plasma spraying or low vacuum plasma spraying, a gas phase deposition such as chemical or physical vapour deposition or modifications thereof, or a slurry technique or combinations of these methods.

12. The method according to any of the preceding claims, wherein in step d. the quality of the restored metallic coating is controlled by non-destructive techniques, preferably selected from the group of: infrared thermography, X-ray fluorescence spectroscopy, ultrasonic or eddy current techniques or combinations thereof.

13. The method according to any of the preceding claims, wherein the component is a gas turbine component, wherein preferably the gas turbine component, at least on the concerned surface region, consists of a Ni, Co, or Fe based superalloy or of a Ti based superalloy.

14. The method according to any of the preceding claims, wherein the metallic coating (2) consists of one or more layers, which are distinguished by their chemical or physical properties, and wherein preferably at least one layer of the metallic coating is of MCrAI(X) type, where: M is an element selected from the group containing Ni, Co, Fe and combinations thereof; X is an element selected from the group consisting of Y, Ta, Si, Hf, Ti, Zr, B, C and combinations thereof and/or wherein preferably at least one layer of the metallic coating is an aluminide, noble-metal-aluminide, noble metal-nickel-aluminide and combinations thereof.

15. The method according to any of the preceding claims, wherein the geometry of the counter electrode is configured and arranged such that the distance between the counter electrode and the component is larger in locations where less coating shall be removed and in locations where less coating shall be removed the size and/or the structure/surface and/or the position and/or the topology and/or the grid structure/width of the counter electrode is adjusted.

16. The method according to any of the preceding claims, wherein prior to step a. a ceramic coating present on the surface of the metallic coating (2) is removed, preferably mechanically removed.

17. The method according to any of the preceding claims, wherein in step c. the new coating is applied using a galvanic deposition process and the amount of the new coating applied is a function of the identification or determination of step a., wherein preferably the geometry of the counter electrode is configured and arranged such that the distance between the counter electrode and the component is larger in locations where less coating shall be reconstituted and in locations where coating shall be reconstituted the size and/or the structure/surface and/or the position and/or the topology and/or the grid structure/width of the electrode is adjusted, and wherein most preferably, if for the removal of the coating an electrolytic process was used with a specifically configured and arranged counter electrode, that same counter electrode geometry is used for the deposition.

## Patentansprüche

1. Verfahren zur Wiederherstellung einer Metallbeschichtung (2) eines Bauteils (1), wobei die Beschichtung (2) einen abgenutzten Abschnitt (3, 4) und das Verfahren folgende Schritte umfasst:
a. Lokalisierung des abgenutzten Abschnitts (3, 4) auf dem Bauteil (1), wobei die Lokalisierung durch die Anwendung eines oder mehrerer zerstörungsfreier Verfahren erfolgt;
b. Entfernung im Wesentlichen nur des abgenutzten Abschnitts (3, 4) entsprechend der Lokalisierung in Schritt a, wobei die Entfernung mittels eines Elektrolytverfahrens erfolgt, das folgende Schritte umfasst:
b1. Eintauchen des Bauteils in ein elektrisch leitfähiges Flüssigkeitsbad;
b2. elektrisches Kontaktieren des Bauteils und einer Gegenelektrode, die in dem Bad eingetaucht sind;
b3. Anlegen eines Potentials zwischen dem Bauteil und der Gegenelektrode, so dass das Bauteil als Anode und die Gegenelektrode als Kathode dient;
b4. Steuern des Potentials zwischen der Anode und der Kathode sowie Messen des Stroms zwecks Überwachung der Beschichtungsentfernung oder Steuern des Stroms zwischen der Anode und der Kathode sowie Messen der Spannung zwecks Überwachung der Beschichtungsentfernung;
und
b5. Stoppen der Beschichtungsentfernung in Schritt b4. in Abhängigkeit von der Überwachung der Beschichtungsentfernung;
wobei die Geometrie und der Werkstoff der Gegenelektrode zur Elektrolytentfernung in Schritt b. dazu bestimmt sind, die Metallbeschichtung (2) entsprechend der Lokalisierung in Schritt a. selektiv zu entfernen;
c. Aufbringen der neuen Metallbeschichtung (7) auf eine Weise, dass die in Schritt b. entfernte Beschichtung mindestens ersetzt wird.

2. Verfahren nach Anspruch 1, wobei - wo immer auf dem Bauteil (1) Metallbeschichtung (2) vorhanden ist - diese mindestens teilweise in Schritt b. entfernt wird, was zu einer mindestens teilweisen Verringerung der Dicke der gesamten Metallbeschichtung (2) des Bauteils infolge des Schrittes b. führt.

3. Verfahren nach Anspruch 1 oder 2, das nach dem Schritt c. überdies den folgenden Schritt d. umfasst:
d. Prüfen der Güte der wiederhergestellten Metallbeschichtung (2).

4. Verfahren nach Anspruch 1, 2 oder 3, wobei der Schritt a. zudem die Bestimmung des Zustands abgenutzter (3, 4) oder nicht abgenutzter oder abgenutzter (3, 4) und nicht abgenutzter Abschnitte der Metallbeschichtung (2) umfasst.

5. Verfahren nach einem der vorstehenden Ansprüche, wobei die Bestimmung in Schritt a. mindestens teilweise in Anwendung eines oder mehrerer zerstörungsfreier Verfahren durchgeführt wird, die aus der Gruppe bestehend aus Infrarotthermographie, Röntgenfluoreszenzspektroskopie, Ultraschall- oder Wirbelstromverfahren oder Kombinationen davon ausgewählt werden.

6. Verfahren nach einem der vorstehenden Ansprüche, wobei der Umfang der zu ersetzenden Metallbeschichtung (2) überdies an mindestens einem repräsentativen Bauteil mittels zerstörender Verfahren, wie z.B. metallographischer Untersuchungen, bestimmt wird.

7. Verfahren nach einem der vorstehenden Ansprüche, wobei das elektrisch leitfähige Flüssigkeitsbad eine saure wässrige Lösung ist, die vorzugsweise HCl als Hauptwirkstoff enthält, wobei die Konzentration von HCl vorzugsweise im Bereich zwischen 2-30 Masse-% liegt.

8. Verfahren nach einem der vorstehenden Ansprüche, wobei das elektrisch leitfähige Flüssigkeitsbad eine Temperatur zwischen der Raumtemperatur und 80°C aufweist und/oder einen oder mehrere der folgenden zusätzlichen Bestandteile enthält: Beschleuniger, Inhibitoren, pH-Puffer, Antiabsetzmittel, Entschäumer, Dispergiermittel, Netzmittel, Tenside und Stabilisatoren.

9. Verfahren nach einem der vorstehenden Ansprüche, wobei das elektrisch leitfähige Flüssigkeitsbad mindestens dann gerührt wird, wenn das Potential angelegt wird.

10. Verfahren nach einem der vorstehenden Ansprüche, wobei der Umfang und/oder der Zustand und die entsprechende Stelle der gesamten beschichteten Fläche nach oder gleichzeitig mit Schritt b. mittels eines oder mehrerer zerstörungsfreier Verfahren bestimmt werden, die aus der Gruppe bestehend aus Infrarotthermographie, Röntgenfluoreszenzspektroskopie, Ultraschall- oder Wirbelstromverfahren oder Kombinationen davon ausgewählt werden.

11. Verfahren nach einem der vorstehenden Ansprüche, wobei der Umfang der aufgetragenen neuen Beschichtung in Schritt c. von der Bestimmung in Schritt a. abhängt und das Aufbringen der neuen Metallbeschichtung mittels eines thermischen Spritzverfahrens erfolgt, bei dem es sich vorzugsweise um das Hochgeschwindigkeitsflammspritzen, atmosphärische Plasmaspritzen, Vakuumplasmaspritzen oder Niedervakuumplasmaspritzen, eine Gasphasenabscheidung, wie z.B. eine chemische oder physikalische Dampfabscheidung oder Modifizierungen davon, oder eine Schlickertechnik oder Kombinationen dieser Verfahren handelt.

12. Verfahren nach einem der vorstehenden Ansprüche, wobei die Güte der wiederhergestellten Metallbeschichtung in Schritt d. mittels zerstörungsfreier Verfahren geprüft wird, die aus der Gruppe bestehend aus Infrarotthermographie, Röntgenfluoreszenzspektroskopie, Ultraschall- oder Wirbelstromverfahren oder Kombinationen davon ausgewählt werden.

13. Verfahren nach einem der vorstehenden Ansprüche, wobei es sich bei dem Bauteil um ein Gasturbinenbauteil handelt, das vorzugsweise mindestens an der betreffenden Oberfläche aus einer Ni-, Co- oder Fe-basierten Superlegierung oder einer Ti-basierten Superlegierung besteht.

14. Verfahren nach einem der vorstehenden Ansprüche, wobei die Metallbeschichtung (2) aus einer oder mehreren Schichten besteht, die sich durch ihre chemischen oder physikalischen Eigenschaften unterscheiden, und wobei vorzugsweise mindestens eine Schicht der Metallbeschichtung dem Typ MCrAI(X) entspricht, wobei: M ein aus der Gruppe bestehend aus Ni, Co, Fe und Kombinationen davon gewähltes Element ist; X ein aus der Gruppe bestehend aus Y, Ta, Si, Hf, Ti, Zr, B, C und Kombinationen davon gewähltes Element ist und/oder wobei es sich vorzugsweise bei mindestens einer Schicht der Metallbeschichtung um ein Aluminid, Edelmetallaluminid, Edelmetall-Nickelaluminid und Kombinationen davon handelt.

15. Verfahren nach einem der vorstehenden Ansprüche, wobei die Geometrie der Gegenelektrode so gestaltet und angeordnet ist, dass der Abstand zwischen der Gegenelektrode und dem Bauteil an Orten größer ist, wo weniger Beschichtung entfernt werden soll, wobei die Größe, die Struktur/Fläche, die Position, die Topologie und/oder die Gitterstruktur/-weite der Gegenelektrode an Orten, wo weniger Beschichtung entfernt werden soll, angepasst wird.

16. Verfahren nach einem der vorstehenden Ansprüche, wobei eine auf der Fläche der Metallbeschichtung (2) vorhandene Keramikbeschichtung vor Schritt a. entfernt wird, und zwar vorzugsweise mechanisch entfernt wird.

17. Verfahren nach einem der vorstehenden Ansprüche, wobei die neue Beschichtung in Schritt c. mittels eines galvanischen Abscheideprozesses aufgebracht wird und der Umfang der neuen Beschichtung von der Bestimmung in Schritt a. abhängt, wobei die Geometrie der Gegenelektrode vorzugsweise so gestaltet und angeordnet ist, dass der Abstand zwischen der Gegenelektrode und dem Bauteil an Orten größer ist, wo weniger Beschichtung wiederhergestellt werden soll, wobei die Größe, die Struktur/Fläche, die Position, die Topologie und/oder die Gitterstruktur/-weite der Elektrode an Orten, wo Beschichtung wiederhergestellt werden soll, angepasst wird, und - wenn zur Entfernung der Beschichtung ein Elektrolytverfahren mit einer speziell gestalteten und angeordneten Gegenelektrode angewandt worden ist - für die Abscheidung vorzugsweise dieselbe Geometrie der Gegenelektrode verwendet wird.

## Revendications

1. Procédé de restauration d'un revêtement métallique (2) d'un composant (1), dans lequel le revêtement (2) inclut une partie consommée (3, 4), le procédé comprenant les étapes suivantes :
a. l'identification de la partie consommée (3, 4) en fonction de son emplacement sur le composant (1), l'identification étant effectuée à l'aide d'une ou plusieurs techniques non destructives ;
b. le retrait essentiellement uniquement de la partie consommée (3, 4) en fonction de l'emplacement identifié à l'étape a., le retrait étant effectué à l'aide d'un procédé électrolytique comprenant les étapes suivantes :
b1. l'immersion du composant dans un bain liquide électroconducteur ;
b2. la mise en contact électrique du composant et d'une contre-électrode, lesquels sont immergés dans ledit bain ;
b3. l'application d'un potentiel entre le composant et ladite contre-électrode, de sorte que le composant fonctionne comme une anode et la contre-électrode comme une cathode ;
b4. la commande du potentiel entre anode et cathode et mesure du courant afin de surveiller le retrait du revêtement ou commande du courant entre l'anode et la cathode et mesure de la tension afin de surveiller le retrait du revêtement ; et
b5. l'arrêt du retrait du revêtement de l'étape b4. sur la base de la surveillance du retrait du revêtement ;
dans lequel à l'étape b., la géométrie et le matériau de la contre-électrode pour le retrait électrolytique sont configurés et agencés pour retirer sélectivement le revêtement métallique (2) en fonction de l'emplacement identifié à l'étape a.,
c. l'application d'un nouveau revêtement métallique (7) de manière à au moins compenser le revêtement retiré à l'étape b.

2. Procédé selon la revendication 1, dans lequel, partout où le revêtement métallique (2) est présent sur le composant (1), il est au moins partiellement retiré à l'étape b.,
conduisant à une réduction au moins partielle de l'épaisseur de l'ensemble du revêtement métallique (2) sur le composant (1) à l'issue de l'étape b.

3. Procédé selon les revendications 1 ou 2, comprenant en outre, après l'étape c., l'étape d. suivante :
d. la vérification de la qualité du revêtement métallique restauré (2).

4. Procédé selon les revendications 1, 2 ou 3, dans lequel l'étape a. comprend en outre une détermination de l'état soit des parties consommées (3, 4) ou non consommées, soit des parties consommées (3, 4) et non consommées du revêtement métallique (2).

5. Procédé selon l'une quelconque des revendications précédentes, dans lequel l'identification ou la détermination de l'étape a. est effectuée au moins en partie à l'aide d'une ou plusieurs techniques non destructives, choisies dans le groupe suivant : thermographie infrarouge, Spectroscopie de fluorescence des rayons X, techniques à base d'ultrasons ou de courants de Foucault ou leurs combinaisons.

6. Procédé selon l'une quelconque des revendications précédentes, dans lequel la quantité de revêtement métallique (2) à remplacer est également déterminée sur au moins un composant représentatif par des techniques destructives telles que, mais non limitées à, des analyses métallographiques.

7. Procédé selon l'une quelconque des revendications précédentes, dans lequel le bain liquide électroconducteur est une solution acide aqueuse, comprenant de préférence du HCl comme principal constituant actif, la concentration de HCl se situant de préférence dans la plage de 2 à 30 % en masse.

8. Procédé selon l'une quelconque des revendications précédentes, dans lequel le bain liquide électroconducteur a une température comprise entre la température ambiante et 80°C, et/ou dans lequel le bain liquide électroconducteur contient un ou plusieurs des constituants supplémentaires suivants : accélérateurs, inhibiteurs, tampons pH, agents suspenseurs, agents antimoussants, dispersants, agents mouillants, tensioactifs et stabilisants.

9. Procédé selon l'une quelconque des revendications précédentes, dans lequel le bain liquide électroconducteur est agité au moins lorsque le potentiel est appliqué.

10. Procédé selon l'une quelconque des revendications précédentes, dans lequel à la suite de l'étape b. ou simultanément, la quantité, et/ou l'état et l'emplacement associé de la totalité de la surface revêtue sont déterminés à l'aide d'une ou plusieurs techniques non destructives, choisies de préférence dans le groupe suivant : thermographie infrarouge ; spectroscopie de fluorescence des rayons X, techniques à base d'ultrasons ou de courants de Foucault ou leurs combinaisons.

11. Procédé selon l'une quelconque des revendications précédentes, dans lequel à l'étape c., la quantité du nouveau revêtement appliqué est fonction de l'identification ou de la détermination de l'étape a. et l'application du nouveau revêtement métallique se fait au moyen d'une technique de pulvérisation thermique, la technique de pulvérisation thermique étant de préférence une pulvérisation d'oxy-combustible à haute vitesse, une projection de plasma sous pression atmosphérique, une projection de plasma sous vide ou une projection de plasma sous vide peu poussé, un dépôt en phase gazeuse tel qu'un dépôt chimique ou physique en phase vapeur ou des modifications de ceux-ci, ou une technique à base de boues ou des combinaisons de ces procédés.

12. Procédé selon l'une quelconque des revendications précédentes, dans lequel à l'étape d. la qualité du revêtement métallique restauré est contrôlée à l'aide de techniques non destructives, choisies de préférence dans le groupe suivant : thermographie infrarouge, spectroscopie de fluorescence des rayons X, techniques à base d'ultrasons ou de courants de Foucault ou des combinaisons de celles-ci.

13. Procédé selon l'une quelconque des revendications précédentes, dans lequel le composant est un composant de turbine à gaz, le composant de turbine à gaz étant constitué de préférence, au moins dans la région de la surface concernée, d'un superalliage à base de Ni, Co, ou Fe ou d'un superalliage à base de Ti.

14. Procédé selon l'une quelconque des revendications précédentes, dans lequel le revêtement métallique (2) est constitué d'une ou plusieurs couches qui se distinguent par leurs propriétés chimiques ou physiques, et dans lequel, de préférence, au moins une couche du revêtement métallique est du type MCrAl(X), où : M est un élément choisi dans le groupe contenant Ni, Co, Fe et leurs combinaisons ; X est un élément choisi dans le groupe constitué de Y, Ta, Si, Hf, Ti, Zr, B, C et leurs combinaisons et/ou dans lequel, de préférence, au moins une couche du revêtement métallique est un aluminure, un aluminure de métal noble, un aluminure de métal noble et de nickel et leurs combinaisons.

15. Procédé selon l'une quelconque des revendications précédentes, dans lequel la géométrie de la contre-électrode est configurée et agencée de sorte que la distance entre la contre-électrode et le composant est plus importante aux emplacements où une plus faible quantité de revêtement doit être retirée et aux emplacements où une plus faible quantité de revêtement doit être retirée, la dimension et/ou la structure ou la surface et/ou la position et/ou la topologie et/ou la structure ou la largeur de grille de la contre-électrode sont ajustées.

16. Procédé selon l'une quelconque des revendications précédentes, dans lequel avant l'étape a., un revêtement de céramique présent à la surface du revêtement métallique (2) est retiré, de préférence retiré mécaniquement.

17. Procédé selon l'une quelconque des revendications précédentes, dans lequel à l'étape c., le nouveau revêtement est appliqué au moyen d'un procédé de dépôt galvanique et la quantité du nouveau revêtement appliqué est fonction de l'identification ou de la détermination de l'étape a., dans lequel de préférence, la géométrie de la contre-électrode est configurée et agencée de sorte que la distance entre la contre-électrode et le composant soit plus importante aux emplacements où une quantité plus faible de revêtement doit être reconstituée et aux emplacements où le revêtement doit être reconstituée, la dimension et/ou la structure ou la surface et/ou la position et/ou la topologie et/ou la structure ou la largeur de grille de l'électrode sont ajustées, et dans lequel de manière préférée entre toutes, si, pour le retrait du revêtement, un procédé électrolytique a été utilisé avec une contre-électrode spécifiquement configurée et agencée, cette même géométrie de contre-électrode est utilisée pour le dépôt.
